

May 4, 1948.

R. T. HURLEY

2,440,952

METHOD OF MAKING PROJECTILES

Original Filed April 16, 1938



BY

INVENTOR.  
*Roy T. Hurley*  
F. Bascom Smith  
ATTORNEY.

## UNITED STATES PATENT OFFICE

2,440,952

## METHOD OF MAKING PROJECTILES

Roy T. Hurley, Westport, Conn., assignor to  
Bendix Aviation Corporation, South Bend, Ind.,  
a corporation of Delaware

Original application April 16, 1938, Serial No.  
202,399. Divided and this application July 29,  
1942, Serial No. 452,709

## 1. Claim. (Cl. 22—204)

1

This invention relates to projectiles and more particularly to projectiles of the type having a rotating band and to methods and means for fixing the rotating band thereto.

This application is a division of copending application Serial No. 202,399, for "Projectiles and methods of making the same," filed April 16, 1938, now Patent No. 2,310,915.

In the methods heretofore proposed for securing a rotating band to a projectile, an oversized ring of soft metal is generally pressed into a dovetail groove in the projectile blank by applying compressive pressure to reduce the diameter of said ring and conform the same to the shape of the groove. The high pressure which is necessarily applied to conform the soft metal band to the shape of the groove distorts the metal and sets up internal stresses within the finished rotating band which tend to weaken the same. Often, as a result of this weakness or because of inadequate compression of the metal ring to completely fill the groove, the joint between the projectile blank and the rotating band is not gas-tight. Accordingly, gas leakage frequently occurs between the band and the projectile when the same are fired from a gun, thereby decreasing the efficiency of the explosive charge and causing the projectile to fall short of its intended target. Furthermore, the leakage of the high pressure gases of explosion between the rotating band and the projectile tends to loosen the former to such an extent that the same will be thrown from the projectile by centrifugal forces acting thereon as the rapidly rotating shell leaves the gun. The loss of the rotating band affects the trajectory of the projectile and, in addition, imperils the personnel in the vicinity of the gun. Because of the necessity for distorting the metal of the rotating band in the methods heretofore employed, the hardness and types of metals which may be employed in practicing said methods is unduly restricted.

Accordingly, one of the objects of the present invention is to provide a novel method for applying a rotating band to a projectile in such a manner that the foregoing disadvantages are obviated.

Another object of the invention is to provide a novel method for applying a rotating band to a projectile whereby said band is caused to become, in effect, an integral part of the projectile.

A further object is to provide a novel method of applying a rotating band to a projectile, which method permits of the use of metals having a wider range of properties such as hardness, ductility, melting point, etc.

2

Still another object is to provide novel means for carrying out the novel method comprehended by the invention, said means being so constituted as to compensate for the thermal expansion of the projectile during the application of the rotating band thereto.

The above and further objects and novel features of the invention will more fully appear from the following detailed description when the same is taken in connection with the accompanying drawings. It is to be expressly understood, however, that the drawings are for the purpose of illustration only and are not designed as a definition of the limits of the invention, reference being had primarily for this latter purpose to the appended claim.

In the drawings, wherein like reference characters refer to like parts throughout the several views,

20 Fig. 1 is a longitudinal sectional view taken substantially along line 1—1 of Fig. 2, showing one form of the novel apparatus comprehended by the present invention, said apparatus being shown in operative position on a projectile;

25 Fig. 2 is a transverse sectional view taken substantially along line 2—2 of Fig. 1; and,

Fig. 3 is a plan view of a completed projectile.

In the illustrated embodiment, one form of means suitable for carrying out the novel process 30 of the invention is shown as comprising a mold 4 which completely encircles a portion of the projectile blank 5 and engages the periphery of the latter on opposite sides of an annular groove 6 provided in said blank for positioning a rotating band 7 (Fig. 3). Mold 4 is provided with a groove 8 which is adapted to register and cooperate with groove 6 to form an annular channel of the same size and shape as the desired rotating band 7. Mold 4 is preferably split along the extension of

40 a horizontal diameter of projectile 5, into two separable sections 4a and 4b, the former, as shown, being the upper section and having a funnel or cup-shaped opening 9 therein, which communicates with the channel formed by grooves 6 and 8.

45 Means are provided for tightly clamping mold sections 4a and 4b to each other around projectile 5 and in the illustrated embodiment said means comprise a pair of arms 10 and 11 (Fig. 2) pivotally secured to opposite sides of section 4b by means of pins 12 and 13, respectively. Said arms are adapted to pivot in the direction of section 4a and to have the free ends thereof extend over slightly concaved shoulders 14 formed on opposed sides of said section. Cam levers 15 and 55 16 are pivotally secured to the free ends of arms

10 and 11, respectively, for rotation relative to the latter. When said levers are pivoted upwardly and inwardly to the positions shown in Fig. 2, the cam-shaped portions of said levers bear against shoulders 14 and apply a pressure thereto in the direction of section 4b. Sections 4a and 4b may be thus tightly clamped to each other and to projectile blank 5.

In practicing the novel method comprehended by the present invention for applying rotating band 7 to projectile blank 5, the latter is first positioned in mold 4 so that the edges of groove 6 coincide with or are suitably positioned relative to the edges of groove 8. Arms 10 and 11 are pivoted in the direction of section 4a until the cam surfaces of levers 15 and 16 are directly over shoulder 14 and then said levers are pivoted upwardly and inwardly to cause a pressure to be applied to shoulders 14, thereby clamping section 4a to section 4b. A metallic slug 17 from which rotating band 7 is to be formed is then inserted into opening or conduit 9 and the whole is placed in a furnace having a reducing atmosphere, such as in a hydrogen furnace. The temperature within the furnace is then raised until slug 17 melts and the molten metal flows into the channel formed by grooves 6 and 8. The metal, preferably a copper alloy, from which slug 17 is made, is so chosen that when the same is in a molten state, it will wet the surfaces of groove 6. Thus, when the mold and projectile blank are permitted to cool, the rotating band is cast in place and fused to the steel projectile so as to form an integral part thereof. It will be understood that groove 6 may be dovetailed, if desired, but this is not necessary to secure an adequate bond between the band and projectile when practicing the method of the present invention.

Slug 17 which is preferably composed of copper or a copper alloy determines the composition of mold 4 since the latter must be formed from, or at least coated with, a metal, such as stainless steel, which will not be wet by the metal constituting the slug when the latter is in a molten state. In other words, mold 4 must be formed from a metal which will not fuse with the copper or other suitable metal of slug 17 in the reducing atmosphere of the furnace. Accordingly, when the liquefied metal flows into channel 6-8, it will become fused or brazed only to the surface of groove 6, thereby rigidly fixing the subsequently solidified band 7 to projectile 5 and permitting the ready removal of mold sections 4a and 4b after solidification.

In order to insure against any possible leakage of the molten metal between the engaging surfaces of mold 4 and shell body 5, the former is made of metal which preferably has a coefficient of thermal expansion equal to or slightly less than the coefficient of thermal expansion of body 5. It has been determined that, if the projectile is made of a mild steel having a coefficient of thermal expansion of about .0000063 inch per degree Fahrenheit, for example, the mold may be made of a stainless steel commercially known as Carpenter No. 2 which has a chromium content of from 12 to 14 per cent and a carbon content of .3 per cent and which has a coefficient of thermal expansion of about .0000056 inch per degree Fahrenheit. A suitable metal which may be employed in making the mold is commercially known as Firth Sterling AA and is a stainless

steel having a chromium content of from 13 to 14 per cent and a very low carbon content and having a coefficient of thermal expansion of about .0000059 inch per degree Fahrenheit. To further insure against leakage of the molten metal, the surfaces of mold 4 which are in contact with the periphery of projectile 5, and the surfaces of sections 4a and 4b which engage each other when said sections are clamped in operative position may be coated or plated with a silicate of soda or a graphite paint. The inclusion of a film of said plating or paint between the contacting surfaces effectively prevents any leakage of the molten metal between said surfaces.

There is thus provided a novel method for producing a novel projectile having a rotating band which is fused to the projectile body. The fusion of band to body produces a firm bond therebetween and eliminates the possibility of leakage of gases of explosion between the band and the projectile body and the danger of said band being thrown from the shell by centrifugal forces. The efficiency and accuracy of the firing is thereby increased and the dangers to the personnel are materially reduced.

Although only a single embodiment of this invention has been illustrated and described, it is to be expressly understood that the same is not limited thereto, but that various changes may be made therein. For example, metals having properties different from those of copper or a copper alloy may be employed, if desired, for the rotating band and a metal other than stainless steel may be utilized in making the mold. Changes in the design and arrangement of parts may also be made without departing from the spirit and scope of the invention, as will now be understood by those skilled in the art. For a definition of the limits of the invention, reference will be had primarily to the appended claim.

#### What is claimed is:

The method of applying an annular projecting rotating band to a projectile having a mild steel body that comprises sealing about the projectile a mold comprising high chromium stainless steel having an annular groove in register with the groove in the projectile, and filling the cooperating grooves with a molten metallic material comprising copper whereby there is formed a ring adherent to the projectile but not to the mold.

ROY T. HURLEY.

#### REFERENCES CITED

55 The following references are of record in the file of this patent:

#### UNITED STATES PATENTS

| Number    | Name            | Date           |
|-----------|-----------------|----------------|
| 116,408   | Britten         | June 27, 1871  |
| 478,020   | Pollard         | June 28, 1892  |
| 1,153,197 | Craig           | Sept. 14, 1915 |
| 1,168,062 | Deppeeler       | Jan. 11, 1916  |
| 1,347,481 | Jeffries        | July 20, 1920  |
| 1,703,442 | Giles           | Feb. 26, 1929  |
| 1,809,872 | Soderberg       | June 16, 1931  |
| 1,922,598 | Morin           | Aug. 15, 1933  |
| 1,991,539 | Boegehold       | Feb. 19, 1935  |
| 2,099,208 | Horsfall et al. | Nov. 16, 1937  |
| 2,150,045 | Ahler           | Mar. 7, 1939   |
| 2,275,503 | Brown           | Mar. 10, 1942  |
| 2,339,141 | Brown           | Jan. 11, 1944  |